

No. 769,337.

PATENTED SEPT. 6, 1904.

G. H. CLAMER.

JOURNAL BEARING.

APPLICATION FILED MAR. 10, 1903.

NO MODEL.



Fig. 1



Fig. 2



Fig. 3

Witnesses:  
C. H. Meeks  
Frank E. French

Inventor:  
William H. Clamer  
By  
Augustine S. Langdon  
Attorney

## UNITED STATES PATENT OFFICE.

GUILLIAM H. CLAMER, OF PHILADELPHIA, PENNSYLVANIA.

## JOURNAL-BEARING.

SPECIFICATION forming part of Letters Patent No. 769,337, dated September 6, 1904.

Application filed March 10, 1903. Serial No. 147,059. (No model.)

*To all whom it may concern:*

Be it known that I, GUILLIAM H. CLAMER, a citizen of the United States, residing at Philadelphia, in the county of Philadelphia and State 5 of Pennsylvania, have invented a certain new and useful Railway Axle-Bearing, of which the following is a specification.

The object of the present invention is to provide a very efficient railway axle-bearing at 10 an extremely low cost.

To this and other ends hereinafter set forth the invention, stated in general terms, comprises a railway axle-bearing consisting of the combination with a stiff metal back of a 15 homogeneous self-fitting filling possessed of a high melting-point and such as it is impossible to melt out by temperature induced by friction of service and the bearing as a whole possessed of sufficient mechanical strength for 20 resisting thrusts and the like; and the invention further comprises the improvements to be presently described and finally claimed.

The nature, characteristic features, and scope of my invention will be more fully understood from the following description, taken 25 in connection with the accompanying drawings, forming part hereof, and in which—

Figure 1 is a perspective view of the filling. Fig. 2 is a similar view of the back, and Fig. 30 3 is a sectional view showing the parts assembled.

In the drawings the filling *c* consists of homogeneous metal possessed of a high melting-point and of a quality which may be designated 35 "self-fitting" in the sense that it is soft enough to adjust itself to the journal. At the same time its high melting-point removes all possible danger of its being fused or otherwise forced out of position. Such a metal is 40 not possessed of sufficient mechanical strength to resist end thrust and equivalent strains.

*a* is the stiff back with which the filling *c* is combined and which imparts to the bearing the necessary resistance to end thrust and 45 other strains and which need not be of anti-friction metal and may consist of a comparatively inexpensive metal, as iron.

The railway-bearing as a whole is comparatively light and inexpensive and consists of

two parts, one of which is homogeneous, self-fitting, and of high melting-point, but too weak to withstand the strains and thrusts to which a railway-bearing is subjected, and the other of which imparts the necessary strength for opposing the strains and thrusts. 50

As shown, the filling is formed with overhanging portions *b*, which extend over the ends of the back and serve to take up the end or collar wear, and the complemental lugs *e* and recesses *b* constitute means for securing the 55 parts to place; but these are details of construction which are not of the essence of the invention. As an example of metal from which to make the filling reference is made to an alloy consisting, essentially, of copper and lead in the proportions of from thirty to seventy per cent. of copper and thirty to seventy per cent. of lead, although it may contain in addition impurities or a small quantity of tin or other elements which may be added to improve 60 its homogeneity or casting properties. Such an alloy possesses a high melting-point—about 1500° Fahrenheit—and it is impossible to melt it out of a railway-bearing at a temperature induced by friction. Furthermore, it is so soft 65 that it is self adjusting or fitting and may be put into service without fear of heating. At the same time it exhibits a greatly-diminished rate of wear. Iron or steel is an example of 70 the material suitable for the stiff back, and it is possessed of sufficient strength for resisting the thrusts and strains to which the bearing is subjected. 75

It will be obvious to those skilled in the art to which my invention appertains that modifications may be made in detail without departing from the spirit thereof. Hence I do not limit myself to the precise construction and arrangement of parts hereinabove set forth, and illustrated in the accompanying 80 drawings; but,

Having thus described the nature and objects of my invention, what I claim as new, and desire to secure by Letters Patent, is—

1. A railway axle-bearing consisting of the 95 combination with a stiff metal back of a homogeneous self-fitting filling possessed of a high melting-point and such as it is impossible to

melt out by temperature induced by friction and the bearing as a whole having sufficient mechanical strength to resist thrusts and the like, substantially as described.

5 2. A railway axle-bearing consisting of the combination with a stiff metal back of a homogeneous self-fitting filling having a melting-point above 800° and such as it is impossible to melt out by temperature induced by friction and the bearing as a whole possessed of sufficient mechanical strength to resist thrusts, substantially as described.

10 3. A railway axle-bearing consisting of the combination with a stiff metal back of a self-fitting filling consisting of an alloy composed essentially of copper and lead in proportions of from thirty to seventy per cent. copper

and thirty to seventy per cent. lead, substantially as described.

4. A railway axle-bearing consisting of the combination with a simple casting consisting of a stiff metal back of a filling consisting of an alloy composed of essentially copper and lead in proportions of thirty to seventy per cent. copper and thirty to seventy per cent. lead, substantially as described.

In testimony whereof I have hereunto signed my name in the presence of two subscribing witnesses.

GUILLIAM H. CLAMER.

Witnesses:

K. M. GILLIGAN,  
W. J. JACKSON.